

## UNITED STATES PATENT OFFICE.

FREDERICK M. BECKET, OF NEW YORK, N. Y., ASSIGNOR TO ELECTRO METALLURGICAL COMPANY, OF NEW YORK, N. Y., A CORPORATION OF WEST VIRGINIA.

## WEAR-RESISTING CHROME-IRON MEMBER.

No Drawing.

Application filed September 7, 1922. Serial No. 586,783.

*To all whom it may concern:*

Be it known that I, FREDERICK M. BECKET, a citizen of the United States, residing at New York, in the county of New York and State of New York, have invented certain new and useful Improvements in Wear-Resisting Chrome-Iron Members, of which the following is a specification.

This invention relates to the manufacture from chrome-iron alloys of members characterized by high surface hardness together with resistance to corrosion, oxidation at elevated temperatures, and attack by corrosive vapors or liquids. Such members as are comprised within my invention are sufficiently non-brittle, strong, and homogeneous to adapt them to stand the strains and impacts to which wearing members are ordinarily subjected.

United States Patent 1,245,552, issued to me on Nov. 6, 1917, discloses chrome-iron alloys containing 1.5% to 3% of carbon, which are exceedingly hard and tough, and resistant to oxidation even at very high temperatures. These properties adapt them for use as wearing members, even under corrosive conditions, but the workability of the compositions in question is not sufficiently good to permit the ready shaping of the alloy into the desired form.

In the application filed by the present applicant and Charles E. McQuigg on March 3, 1922, Serial No. 540,885, non-corroding chrome-iron compositions having a much better workability when heat-treated in the manner set forth therein, are disclosed. The shaping of members from the compositions disclosed in said application is quite readily accomplished, but a higher carbon content is often necessary to develop the maximum hardness and wear-resisting qualities possible for the proportions of iron and chromium present.

In accordance with the present invention, it is possible to produce an alloy adapted by its chromium content to resist corrosion and by its carbon content for easy working, to shape the alloy into the desired form, and then to increase the carbon content to such a figure that the desired hardness and resistance to wear are developed. It will usually be sufficient to increase the carbon content only superficially, giving a case or surface layer of great hardness. This object is attained by subjecting the

shaped member to a suitable carbonizing treatment. The following examples will serve to illustrate the carbonizing operation.

A section of sheet one-sixteenth inch thick, containing 26.60% chromium, 0.80% carbon, 0.10% silicon and 0.39% manganese, the remainder being iron, was packed in a commercial carbonizing material of unknown composition, the material being known in the trade as E. F. Houghton's "Quick Light A", and heated at 900° C. for 108 hours. With this thin material, the entire cross section became carbonized, though doubtless to a varying degree, and a sample representing the entire cross section showed a carbon content of 1.41%. The scleroscopic hardness was materially increased after carbonization.

Another sample having a cross section which roughly resembled a right triangle with a base of about 0.65 inch and an altitude of about 0.5 inch, was heated in the same material at 960° C. for 48 hours. The initial composition of the alloy was: chromium 28.77%, carbon 1.25%, silicon 1.29% and manganese 0.65%, the remainder being iron. After carbonization, the average carbon content of the entire cross section was 1.73%, while a sample of metal taken from the surface contained 1.92% carbon. The surface hardness of this sample was also increased.

The carbonizing compound employed in the specific examples is one commonly used for the hardening of ordinary steels and is regarded as a very active carbonizing material. It is believed that the carbonizing materials now in use for hardening steels are in general also applicable to chromium alloys.

The finished member, if its size and the carbonizing treatment are such that carbonization has not proceeded to the center, may have an interior portion of a composition corresponding to a readily workable material. However, the invention also comprises members such as may result from the carbonization of pieces which even before such treatment had a carbon content so high that they could not be rolled or drawn, or only with difficulty.

Members of the kind described herein have many applications but are particularly suitable for the wearing parts of gauges,

and for bearings, especially the balls and races of ball bearings. When the chromium content is upward of 20%, they may be subjected to high temperatures and to corrosive conditions without losing their usefulness.

I claim:

1. A member which in its regular use is continually subjected to abrasion, composed of case-carbonized chrome-iron.

2. A member which in its regular use is continually subjected to abrasion, composed of case-carbonized chrome-iron of sufficient chromium content to render it non-corroding.

3. A member which in its regular use is continually subjected to abrasion, composed of case-carbonized chrome-iron containing upward of 20% of chromium.

4. A ball-bearing member composed of 20 case-carbonized chrome-iron.

5. A ball-bearing member composed of case-carbonized chrome-iron of sufficient chromium content to render it non-corroding.

6. A case-carbonized ball-bearing member containing upward of 20% chromium.

In testimony whereof, I affix my signature.

FREDERICK M. BECKET.